

## UNITED STATES PATENT OFFICE

RICHARD HAYNN, OF FRANKFORT-ON-THE-MAIN-FECHENHEIM, GERMANY, ASSIGNOR  
TO GENERAL ANILINE WORKS, INC., OF NEW YORK, N. Y., A CORPORATION OF DELA-  
WARE

PROCESS FOR MANUFACTURING PIECE-DYED WOOLEN FABRICS CONTAINING  
EFFECTS OF SILK

No Drawing. Application filed September 10, 1928, Serial No. 305,146, and in Germany September 16, 1927.

The present invention relates to a process of manufacturing piece-dyed woolen fabrics containing effects of silk, more particularly it relates to a process of obtaining clean effects of silk in piece-dyed woolen fabrics.

It is highly desirable, when dyeing woolen fabrics containing effects of silk, that these effects remain clean and do not take on the wool dyestuff.

10 I have now found that this purpose is accomplished if sulfonic acids of organic compounds, capable of precipitating glue and gelatin from an acid solution, are added to the dye baths. The products, described for instance in the U. S. Patents No. 1,237,405, No. 1,796,801 and No. 1,336,759, being condensation products from formaldehyde and phenols or phenol sulfonic acids or sulfonic acids of the naphthalene series and likewise products obtainable by acting with sulfur trioxide on unsaturated higher fatty or hydroxyfatty acids or their esters, are particularly suitable for my process. The addition of these compounds is advantageously carried out during 25 the dyeing process, or, if chromable dyestuffs are used, before afterchroming.

My new process has the further advantage that a greater number of different dyestuffs than was hitherto possible can be employed 30 for dyeing fabrics of this kind. Two-colored effects, especially are produced in a particularly clear state by this process.

In order to further illustrate my invention the following examples are given, but I wish 35 it to be understood that my invention is not limited to the examples given, nor to the exact conditions stated therein.

*Example 1*

40 A woolen fabric containing white effects of silk is dyed in the usual manner with 7% of naphthol blue black S Colour Index No. 246. After boiling for about 1 hour, 10% of 45 a condensation product, prepared according to Example 1 of the U. S. Patent No. 1,336,759, by treating naphthalene-beta-sulfonic acid with formaldehyde, are added to the dye-bath. Then the dyeing is continued at the 50 boiling point for half an hour. Thereafter

the goods are rinsed and dried. The effects of silk remain clean white.

*Example 2*

A woolen fabric containing white effects 55 of silk is dyed in the usual manner with 8% of anthracene acid black ST Colour Index No. 303 with the addition of formic acid. After boiling for about 1 hour, 10% of the product, obtained by acting with sulfur trioxide in the form of fuming sulfuric acid on castor oil as described in U. S. Patent No. 1,796,801, are added. Then the dyeing is continued at the boiling point for half an hour. Thereafter the black dyeing is developed 60 in the known manner and afterchromed, for instance with 2.5% of postassium bichromate, for half-an-hour while hot. The effects of silk remains clean white. 65

I claim:

1. A process for obtaining clean effects of 70 silk in piece-dyed woolen fabrics, which comprises dyeing woolen fabrics containing effects of silk with wool dyestuffs and adding organic sulfonic acid compounds of the group consisting of condensation products of formaldehyde with phenol-sulfonic acids or naphthalene-sulfonic acids and of sulfonation products prepared from sulfur trioxide and unsaturated fatty- or hydroxy fatty acids 75 or their esters to the dye-bath. 80

2. A process for obtaining clean effects of 85 silk in piece-dyed woolen fabrics which comprises dyeing woolen fabrics containing effects of silk with wool dyestuffs and adding organic sulfonic acid compounds, of the group consisting of condensation products of formaldehyde with phenol-sulfonic acids or naphthalene-sulfonic acids and of sulfonation products prepared from sulfur trioxide 90 and unsaturated fatty- or hydroxy fatty acids or their esters to the dye-bath, during the dyeing process. 95

3. A process for obtaining clean effects of 100 silk in piece-dyed woolen fabrics which comprises dyeing woolen fabrics containing effects of silk with chromable wool dyestuffs, adding organic sulfonic acid compounds, of the group consisting of condensation products of formaldehyde with phenol-sulfonic acids or

naphthalene-sulfonic acids and of sulfonation products prepared from sulfur trioxide and unsaturated fatty- or hydroxy fatty acids or their esters to the dye-bath, during the dyeing process and then afterchroming the fabrics.

5 In testimony whereof, I affix my signature.

**RICHARD HAYNN.**

10

15

20

25

30

35

40

45

50

55

60

65